

(No Model.)

C. T. & V. E. MEYER.  
FLOOR COVERING.

No. 252,122.

Patented Jan. 10, 1882.



WITNESSES:

*Chas. Nida.*  
*D. Sedgwick*

BY

INVENTOR:  
*C. T. Meyer*  
*V. E. Meyer*  
*Minn & Co.*  
ATTORNEYS.

# UNITED STATES PATENT OFFICE.

CHARLES T. MEYER AND VICTOR E. MEYER, OF JERSEY CITY, N. J.

## FLOOR-COVERING.

SPECIFICATION forming part of Letters Patent No. 252,122, dated January 10, 1882.

Application filed June 21, 1881. (No model.)

*To all whom it may concern:*

Be it known that we, CHARLES T. MEYER and VICTOR E. MEYER, of Jersey City, in the county of Hudson and State of New Jersey, 5 have invented a new and Improved Floor-Covering, of which the following is a specification.

The object of our invention is to provide a new and improved floor-covering which is more durable and substantial and less apt to crack 10 than the floor-coverings in use heretofore.

The invention consists in a floor-covering made of a fabric covered with a coating or mixture of ground wood or other vegetable fiber, either plain or dyed, with mineral fiber 15 and a binding material, such as copal or other varnish.

In the accompanying drawing cross-sectional elevations of specimens of our improved floor-covering are shown.

20 In carrying out our invention we prepare a mixture of ground wood or other vegetable fiber, which may be plain or dyed and colored in some suitable manner, with some mineral fiber and a binding material, such as copal or

25 other varnish, to which a small proportion of rubber solution is added. The proportions are about as follows: ground wood or other vegetable fiber, fifty parts, in weight; mineral fiber, two hundred parts, in weight; varnish binding material, forty gallons; but we do not limit 30 ourselves to these proportions, but may vary them as circumstances may require. The ground wood or other vegetable fiber is used plain, or is dyed by means of aniline colors or

35 dye-woods or other colors, or colored in any other suitable manner, before being mixed with the varnish. The canvas A or other fabric is first sized in the ordinary manner, and a layer, B, or several layers, B, of the above-described

40 compound are spread on the canvas, and the lower surface of the canvas is painted with oil-

paint or a more diluted compound of the above ingredients.

The coating may be of greater or less thickness, according to the thickness of the canvas, 45 or as the circumstances may require.

The mixture can be spread with a brush or trowel, by machinery, or in any other suitable manner.

If desired, the mixture may consist of varnish 50 and the wood fiber only; but we prefer the compound given above.

A design is printed on this floor-covering in the ordinary manner, or it may be left plain.

We are aware that floor-coverings have been 55 made of canvas covered with a mixture of ground wood, pigment, and varnish; but this we do not claim.

The mineral fiber we propose to use is of 60 the nature of asbestos.

Having thus fully described our invention, we claim as new and desire to secure by Letters Patent—

1. As an improved article of manufacture, a floor-covering made substantially as herein 65 shown and described, and consisting of a layer of canvas or another base, on which a layer or layers of a mixture of ground wood or other vegetable fiber, either plain or dyed or colored, mineral fiber, and a binding material, such as 70 copal or other varnish, are spread, as set forth.

2. A compound for spreading on canvas for floor-coverings, consisting of a mixture of ground wood, either plain or dyed or colored, with copal or other varnish, substantially as 75 herein shown and described, and for the purpose set forth.

CHAS. T. MEYER.  
VICTOR E. MEYER.

Witnesses:

OSCAR F. GUNZ,  
C. SEDGWICK.